

## UNITED STATES PATENT OFFICE

2,311,027

## TEXTILE TREATMENT

William J. Burke, Robert W. Maxwell, and Paul S. Pinkney, Wilmington, Del., assignors to E. I. du Pont de Nemours & Company, Wilmington, Del., a corporation of Delaware

No Drawing. Application November 8, 1940,  
Serial No. 364,850

14 Claims. (Cl. 8—115.5)

This invention relates to the treatment with formaldehyde of textile materials which are reactive thereto. More particularly, it relates to a process for reacting a textile material with formaldehyde without objectionably altering the dye affinity of the textile material.

It has long been known to react textile materials with formaldehyde. Such reaction has been carried out for the purpose of increasing the strength of textiles or to improve their resilience, crease resistance, crush resistance, crimp retention, resistance to shrinking, and to reduce the dry and wet elongation and the extent to which such materials are swelled by water.

Many of these previously known processes are objectionable in that they alter the dye affinity of the textile material.

It is, therefore, an object of the present invention to provide a process for reacting a textile material with formaldehyde without objectionably altering the dye affinity of the textile material.

Other objects of the invention will appear hereinafter.

The objects of this invention may be accomplished, in general, by impregnating a formaldehyde-reactive textile material with the desired quantity of formaldehyde together with an acid-reacting catalyst, drying the impregnated material and heating the same to the desired reaction temperature by immersion in a hot organic liquid bath having a basic reaction, preferably a bath comprising a sufficient quantity of a basic nitrogen-containing material that the bath as a whole is basic in reaction.

The following examples illustrate in great detail the preferred methods of carrying out the process of this invention. It is to be understood, however, that the present invention is not limited to the specific details set forth therein.

## Example I

Skeins of the newly developed crimped viscose rayon yarn described and claimed in United States application, Serial No. 180,976, filed December 21, 1937, by William Hale Charch and William Frederick Underwood, are impregnated with a water solution containing 2% of formaldehyde and 0.2% of ammonium chloride. The skeins of yarn are then centrifuged and dried at room temperature. One of said skeins is immersed in mineral oil at 150° C. for 5 minutes and the other is immersed in tris(β-hydroxyethyl)-amine at 150° C. for 5 minutes. Both skeins are then thoroughly washed to remove all traces of bath liquid. Both skeins show marked improvement in resilience, crease resistance and wet strength. The degree of improvement is about the same in both cases. Samples of each skein are dyed with "Pontamine" Sky Blue 6 BX (Rowe Color Index No. 518). Both sets of samples are

uniformly colored; however, those heated in tris(β-hydroxyethyl)amine are more deeply colored than that heated in mineral oil. Photomicrographs of cross-sections of dyed fibers show that the fibers heated in tris(β-hydroxyethyl)-amine are penetrated more deeply by the dye than are those heated in mineral oil. This shows that a surface layer of the fibers heated in tris(β-hydroxyethyl)amine has been modified less by reaction with formaldehyde than has a similar surface layer of the fibers heated in mineral oil. The fiber cores of both samples are modified substantially to an equal extent in both cases.

## Example II

Five skeins of the yarn described in Example I were impregnated with a water solution containing 13% of formaldehyde and 0.5% of ammonium chloride, centrifuged and dried at room temperature before a fan. The several skeins were heated by immersion for 5 minutes in baths consisting respectively of:

- 1. Aniline having a temperature of 135°—138° C.
- 2. Pyridine having a temperature of 115° C.
- 3. (β-hydroxyethyl)amine having a temperature of 135°—138° C.
- 4. Boiling xylene containing 10% of dimethyl-aniline.
- 5. Boiling n-butyl alcohol containing 4% of sodium butylate.

All five samples showed marked improvement in crease resistance and, upon dyeing with a direct dyestuff showed less loss in dye affinity than samples given comparable crease resistance by treatment with formaldehyde followed by curing in mineral oil.

In accordance with the present invention, any formaldehyde-reactive textile material, particularly a formaldehyde-reactive cellulosic textile material, when impregnated with formaldehyde and an acid reacting catalyst, dried, and then heated by immersion in a hot organic liquid bath having a basic reaction, preferably a bath comprising a sufficient quantity of a basic nitrogen-containing material to render the bath basic in reaction, will produce a uniformly resilient, crush resistant and crease resistant product having improved dyeing characteristics. It is considered that the improved dyeing characteristics result from the fact that the acid reacting catalyst reacts with the basic reacting bath on the surface of the fibers and, therefore, the surface of the fibers remain substantially unmodified. The cores of the fibers, however, are reacted with formaldehyde to substantially the same extent as if the yarn were heated in an inert bath; that is, one which is not basic in character.

As a "formaldehyde-reactive textile material,"

the present invention contemplates the treatment of filaments, yarn, fabrics and the like comprising regenerated cellulose, regenerated protein materials, and low substituted cellulose esters and ethers; i. e., cellulose esters and ethers having at least one unsubstituted hydroxyl group.

The present invention is operative in the treatment of all textile materials which are at all reactive to formaldehyde. In the treatment of such textiles as are less reactive than those specifically referred to above, the treating conditions will, of course, be more drastic.

The term "textile material" includes fibers in the form of loose staple, yarn, fabric, or finished article and filaments in the form of yarn, fabric, or finished article. The fabrics may be knitted, woven, or felted. They may be special types of fabric such as pile fabrics or crepe. Viscose rayon fibers may be treated in the gel state either as staple, rope, or yarn.

The term "acid-reacting catalyst" is intended to include water soluble substances which are acid in reaction, or capable of becoming acid under the conditions of the treatment, or capable of liberating an acid under the conditions of the treatment. Examples are organic carboxylic or sulfonic acids such as oxalic acid, tartaric acid, and benzenesulfonic acid, acid salts of organic acids such as sodium acid tartrate and potassium tetroxalate, mineral acids such as hydrochloric acid, sulfuric acid, and phosphoric acid, acid salts of mineral acids such as sodium bisulfate and dihydrogen sodium phosphate, and salts of strong acids with weak bases which dissociate in water solution to give an acid reaction such as ammonium thiocyanate, ammonium chloride, ammonium bromide, ammonium iodide, ammonium sulfate, hydroxylamine hydrochloride, ferric chloride, calcium chloride, aluminum chloride, etc. The catalyst chosen in any particular case will be the one which is sufficiently powerful to effect the degree of chemical reaction desired between the textile material and the formaldehyde. Because of its cheapness and effectiveness, ammonium chloride is the catalyst which is preferred in the exercise of this invention.

As liquids suitable for use as components of the heating bath in the process of the present invention, there may be used any organic liquid boiling above 70° C. and preferably above 100° C., which bath is basic in reaction. The bath may, of course, be composed of a neutral liquid material which is capable of dissolving substantial quantities of basic materials without reacting therewith, so that the bath as a whole is basic in reaction under the conditions prevailing during the heating step. As examples of suitable liquids which are basic in reaction, the following may be named: Tertiary amines such as tris(β-hydroxyethyl)amine, triallylamine, tris(β-hydroxypropyl)amine, N-butyl bis(β-hydroxyethyl)amine, diethylaminoethanol, phenylmorpholine, pyridine, dimethylaniline, N-phenyl bis(β-hydroxyethyl)amine, N-ethyl-piperidine, N-bis(β-hydroxyethyl)cyclohexylamine, N-hydroxy-ethylmorpholine, tripropylamine, N,N,N',N'-tetramethylene-diamine, N,N-dimethylbenzylamine, quinoline, etc.; secondary amines such as piperidine, bis(β-hydroxyethyl)-amine, piperazine, morpholine, etc.; and primary amines such as aniline, benzylamine, octylamine, etc. These may also be used as basifying agents for baths consisting mainly of neutral organic liquids.

As examples of suitable liquids which are capable of dissolving substantial quantities of basic materials the following may be named: Hydrocarbons such as benzene, toluene, xylene, kerosene, mineral oil, high boiling benzine, trisobutylene, etc.; alcohols such as glycerol, ethylene glycol, butanols, octanols, etc.; hydroxy ethers such as "Cellosolves" and "Carbitols"; ethers such as diisobutyl ether, bis(methoxyethoxyethyl)ether, bis(ethoxyethyl)ether, dioxan, etc. Of course, ethers or other materials which are solvents for cellulose ethers cannot be used as constituents of baths for heating textile materials composed of cellulose ethers.

15 Basic materials suitable for use as solutes to render the liquid bath basic in reaction may be organic or inorganic. The one to be used with any particular liquid will, of course, depend on its solubility in that liquid. Strong in-

20 organic bases such as sodium and potassium hydroxides, sodamide, and sodium alcohohates need be soluble to an extent of at least 0.5%. Weaker inorganic bases should be more soluble, preferably to an extent of at least 2%, so that an effective concentration can be built up. Other basic materials suitable for use as bath basifying agents include ammonia, urea, butyl urea, thiourea, cyanamide, guanidine, hydrazine, hydroxylamine, etc.

25 30 The formaldehyde treating solution may contain desired modifying agents which will improve the resulting product, as long as the modifying agent does not interfere with the reaction between the formaldehyde and the textile material.

35 For example, long chain agents such as glycerol monostearate or sulfonated castor oil may be added to the formaldehyde solution to improve hand and feel of the textile material.

40 However, when such a long chain agent is used and the liquid heating medium used is a solvent for it, it is preferable to saturate the liquid heating medium with the long chain agent so that the agent will be retained by the textile material and not dissolved out by the heating medium.

45 The concentration of formaldehyde to be used in the treating solution varies, of course, with the material under treatment, the nature and concentration of the catalyst, the nature and concentration of modifying agents, the conditions of drying and heating, and the effect desired. For example, for creaseproofing viscose rayon a higher formaldehyde concentration is required than for shrinkproofing the material, other conditions remaining the same. Generally, when the drying and heating conditions are more severe, that is when higher temperatures and longer times are employed, less formaldehyde is required. Thus, if the impregnated material is dried at 100° C. rather than at room temperature, less formaldehyde will be required to give the same final effect. Generally, to obtain comparable effects, less formaldehyde is required when a more strongly acidic catalyst is employed or when a catalyst is used in higher concentrations, than when a more weakly acidic catalyst is employed or when a catalyst is used in lower concentrations. Usually, a concentration of formaldehyde of at least 1% is required to obtain a noticeable effect on cellulosic materials. The upper limit is the concentration at which the particular textile material being treated is made too weak or too brittle for use. As a general rule, the formaldehyde concentration should not exceed 20%. With these facts

in mind, one skilled in the art can readily determine the concentration of formaldehyde which will give optimum results under a given set of other conditions. A high differential in degree of textile modification between the core and the outer surface of the fiber under treatment is favored by using a relatively high concentration of formaldehyde (5% to 20%) in the treating solution and carrying out the reaction at a relatively low temperature, preferably below 110° C.

The catalyst concentration may vary from as low as 0.05% or lower to as high as 1% or higher depending on the potential acidity of the catalyst, the nature of the textile material under treatment, the concentration of formaldehyde employed, the nature and concentration of modifying agents, the drying and heating conditions, and the effect desired. Other conditions remaining the same, an increase in the catalyst concentration or a change from a less to a more strongly acid catalyst results in a greater degree of modification of the textile material. Usually, the selection of the nature and concentration of the catalyst is a matter of balancing catalyst efficiency against tendering which results from the use of acidic materials on many textile materials, particularly cellulosic materials. By reference to the above examples and the following description one skilled in the art can readily select the proper catalyst and concentration to bring about the desired result.

The treating solution may be applied to the textile material in any of several ways. Staple fibers may be dipped in the solution and squeezed or centrifuged to remove excess solution. Yarn may be passed continuously through the solution or it may be dipped in skein form in the solution and then squeezed or centrifuged to remove excess solution. Flat fabrics may be passed through the solution or the solution may be applied from rolls or by spraying and the excess may be removed by squeezing between rolls or by vacuum extracting. Articles, as of clothing, may be dipped in the solution or sprayed. Fabrics or articles of clothing may be treated locally by spraying.

The formaldehyde and catalyst may also be applied in other ways. For example, the textile material may be wet with a solution of the catalyst and then exposed to vapors of formaldehyde, or it may be wet with formaldehyde solution and then exposed to a gaseous catalyst such as hydrochloric acid.

After impregnation with the treating solution the textile material is preferably dried to a water content of about 15% or less before it is subjected to the final heat treatment. This may be carried out in any of several ways. It may be dried in air or in a heated inert liquid such as a hydrocarbon or ether. If it is air dried, the temperature of drying may range from room temperature to 150° C. or higher. Drying at high temperatures in air must be carried out with care so that no part of the textile material is heated after it is dry. Uniformity is favored by vigorous circulation of air in the drying chamber and by use of temperatures below 100° C., and preferably below 50° C. Liquid temperatures up to 250° C. or higher may be used. If a temperature below 100° C. is used, it is usually necessary to boil the drying liquid in order to carry out the water. Consequently, for drying at such temperatures liquids boiling below 100° C. are desirable. However, if they boil below about 70° C., the rate of

drying will generally be too low for practical purposes.

The time of drying depends, of course, on the drying method used. When the air drying method is used, the time required depends on the temperature, circulation of air, and the relative thickness and looseness of the material under treatment. When the hot liquid drying method is used, the time required depends on the nature of the liquid and the temperature used and less on the construction of the material under treatment. In general, with temperatures below 100° C., the air drying method is more rapid and may require as short a time as 2 minutes. When the material under treatment is in a relatively loose condition so that air will circulate through it freely, air drying has an advantage over drying in a hot liquid in that the formaldehyde concentration required for a given degree of modification is much lower and the overall period during which the material is held at the higher liquid temperature is shorter, so that the risk of tendering due to the effect of the acid reacting catalyst at high temperatures is less. At higher temperatures the liquid drying method is generally more rapid due to more efficient heat transfer between the moisture and the heating medium. In general, with other conditions remaining constant, an increase in the drying temperature leads to a greater degree of modification of the textile material.

In order to bring about a reaction between formaldehyde and the textile material within a reasonable time, it is necessary to heat the impregnated and dried material. In this process the heating step is carried out by immersing the textile material in a hot liquid of the nature disclosed above. The temperature of the liquid may be as low as 70° C. or lower, although a much longer heating period is required at such low temperatures. As already pointed out, if a heating temperature below 100° C. is used, that temperature should be the boiling point of the liquid so that water formed by the reaction will be removed efficiently. The temperature of the liquid may range as high as 200° C. or even higher. However, it should be emphasized that at such high temperatures the heating period should be reduced to the neighborhood of 1 minute or less to avoid damaging the textile material. The heating temperature depends on the amount of formaldehyde used, the nature and amount of catalyst, the nature and amount of modifying agent, the temperature of drying, the time of heating, the effect desired, and the nature of the textile material under treatment. It is common knowledge that some textile materials are more susceptible to damage by heat than are others and so require more careful treatment in any heating process. In general, with other conditions remaining constant, an increase in the temperature of the heating liquid leads to a greater degree of modification of the textile material under treatment.

The heating period may be varied from as long as an hour or more at low temperatures, such as 70°-80° C. or lower, to a fraction of a second at higher temperatures, such as 200° C. or higher. When the heating is to be carried on over a period of about a minute or longer, it is advantageous to place the textile material in a perforated container which is lowered into the hot liquid bath and then lifted after the desired length of time. When yarn or fabric is to be

heated at a higher temperature for a shorter period of time, it is advantageous to pass the yarn or fabric continuously through the heating bath at a rate depending on the length of bath travel. With other conditions remaining constant, an increase in the heating period leads to a greater degree of modification of the textile material under treatment.

From the above descriptions, it will be apparent that the drying step and the heating step may be combined into one continuous step. The drying liquid may be used for the subsequent heat treatment. Thus, it is sometimes convenient to prolong the period of immersion in the drying liquid until the reaction between formaldehyde and the textile material has proceeded to the desired point.

After the heating step, it is usually desirable to remove the heating liquid. This may be accomplished simply by washing the textile material with water. Water-insoluble, non-volatile materials may be displaced by a volatile or water-soluble solvent or removed by soaping. It is usually desirable to neutralize any traces of acidic material which may be left in the yarn by washing with a solution of ammonium hydroxide or other mildly alkaline material. The treated material may then be finished in any desired manner such as by application of a softening agent or water repellent agent.

Since it is obvious that many changes and modifications can be made in the above-described details without departing from the nature and spirit of the present invention, it is to be understood that the invention is not to be limited to the said details except as set forth in the following claims.

We claim:

1. In a process for reacting a textile material with formaldehyde, the steps comprising impregnating said material with an aqueous solution of formaldehyde and an acid reacting catalyst, drying said impregnated material, and heating the same to reaction temperature by immersion in a hot organic liquid bath which is basic in reaction.

2. In a process for reacting a textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of a basic nitrogen-containing material that the bath is basic in reaction.

3. In a process for reacting a textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of a basic amino nitrogen-containing material that the bath is basic in reaction.

4. In a process for reacting a textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient

quantity of a basic tertiary amine that the bath is basic in reaction.

5. In a process for reacting a textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of triethanolamine that the bath is basic in reaction.

6. In a process as defined in claim 1 in which the temperature of the liquid bath is maintained between 70° C. and 200° C.

7. In a process as defined in claim 2 in which the temperature of the liquid bath is maintained between 70° C. and 200° C.

8. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in a hot organic liquid bath which is basic in reaction.

9. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of a basic nitrogen-containing material that the bath is basic in reaction.

10. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of a basic amino nitrogen-containing material that the bath is basic in reaction.

11. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of a basic tertiary amine that the bath is basic in reaction.

12. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in a hot organic liquid bath comprising a sufficient quantity of triethanolamine that the bath is basic in reaction.

13. In a process as defined in claim 8 in which the temperature of the liquid bath is maintained between 70° C. and 200° C.

14. In a process as defined in claim 9 in which the temperature of the liquid bath is maintained between 70° C. and 200° C.

WILLIAM J. BURKE.  
ROBERT W. MAXWELL.  
PAUL S. PINKNEY.